

Dec. 14, 1954

R. V. WHITE ET AL  
TURBINE OIL ANTIOXIDANTS

2,697,073

Filed Feb. 7, 1952



INVENTORS  
RALPH V. WHITE  
HENRY D. NORRIS  
BY

Hastings J. Trigg  
AGENT

# United States Patent Office

2,697,073

Patented Dec. 14, 1954

1

2,697,073

## TURBINE OIL ANTIOXIDANTS

Ralph V. White, Pitman, and Henry D. Norris, Woodbury, N. J., assignors to Socony-Vacuum Oil Company, Incorporated, a corporation of New York

Application February 7, 1952, Serial No. 270,301

11 Claims. (Cl. 252—50)

This invention relates broadly to mineral lubricating oils. It is more specifically concerned with mineral lubricating oils having improved resistance to oxidation.

As is well known to those skilled in the art, most lubricating oils are subject to oxidation during use. In the case of highly-refined oils, such as are used to lubricate steam turbines, attack by atmospheric oxygen at elevated temperatures is most pronounced. Such attack occurs especially readily in the presence of catalytic metals, such as iron, copper, and copper alloys, which are encountered in steam turbines. The deleterious results of such oxidation are manifested by the formation of acidic substances, colored oxidation products, and sludge. It will be obvious to those skilled in the art that such conditions cannot be tolerated in such a finely-machined apparatus as a steam turbine.

It has now been found that the oxidation tendencies of mineral lubricating oils can be sharply inhibited by the addition thereto of a novel antioxidant. It has now been discovered that the reaction products of a tetrakis(halomethyl)methane with certain aromatic amines, when added to mineral lubricating oils increases the resistance thereof to oxidation.

Accordingly, it is a broad object of the present invention to provide improved antioxidants. Another object is to provide mineral lubricating oils, such as steam turbine oils, containing effective antioxidants. A specific object is to provide reaction products of a tetrakis(halomethyl)methane with certain aromatic amines. A further specific object is to provide mineral lubricating oils whose tendency to oxidize has been sharply reduced by the addition of small amounts of these reaction products. Other objects and advantages of the present invention will become apparent to those skilled in the art, from the following detailed description.

In general, the present invention provides a mineral lubricating oil containing a small amount, sufficient to inhibit the oxidation tendencies thereof, of the reaction product obtained by reacting a tetrakis(halomethyl)methane with an aromatic primary or secondary amine; using a molar proportion of aromatic amine to tetrakis(halomethyl)methane of between about 2:1 and about 4:1, respectively, in the case of primary aromatic amines, and of about 4:1 in the case of secondary aromatic amines; and at a temperature of between about 180° C. and about 240° C.

The tetrakis(halomethyl)methane reactant employed to make the reaction products of this invention have the structural formula:



wherein X is a bromine, chlorine or iodine atom. Therefore, the reactants of this type which can be employed herein are tetrakis(bromomethyl)methane, tetrakis(chloromethyl)methane, and tetrakis(iodomethyl)methane.

The aromatic amine reactants utilizable herein are the primary aromatic amines and ring-alkylated derivatives thereof, and N-alkyl aromatic amines and ring-alkylated derivatives thereof. The aromatic ring nucleus can be any aromatic hydrocarbon ring. However, the benzene ring is preferred. The amine reactants contemplated herein are those having the general structural formula:

2

HRN—Y—R', wherein R is a hydrogen atom or an alkyl radical having between one and 5 carbon atoms, R' is a hydrogen atom or a primary or secondary alkyl radical having between one and 5 carbon atoms, and Y is an aromatic hydrocarbon ring, preferably a benzene ring. It has been found that amine reactants having tertiary alkyl substituents on the ring do not form reaction products which are effective in the present invention. There must be at least one hydrogen atom on the carbon atom of the alkyl radical which atom is attached to the aromatic nucleus. Non-limiting examples of the aromatic amine reactant are aniline, 1-naphthylamine, p-toluidine, 1-anthrylamine, o-toluidine, p-ethylaniline, o-isopropyl-aniline, p-sec-butylaniline, o-amyylaniline, N-ethyl-aniline, N-t-butylaniline, N-isoamylaniline, N-methyl-o-butylaniline, N-propyl-m-toluidine, N-ethyl-p-toluidine, N-t-amyl-p-isopropylaniline, N-ethyl-2-naphthylamine, N-propyl-4-methyl-1-naphthylamine, N-butyl-6-sec-amyl-2-naphthylamine, 6-methyl-2-naphthylamine, 4-butyl-1-naphthylamine, 5-methyl-2-anthrylamine, 4-propyl-1-anthrylamine, N-isopropyl-3-sec-butyl-1-anthrylamine, N-methyl-4-amy1-9-anthrylamine, 9-phenanthrylamine, and 4-butyl-1-phenanthrylamine.

The molar proportions of tetrakis(halomethyl)methane reactant and amine reactant used to produce the reaction products of this invention depend upon whether the amine reactant is a primary or a secondary amine. A primary aromatic amine can be reacted in a molar proportion of amine reactant to tetrakis(halomethyl)methane reactant of between about 2:1, respectively, and about 4:1, respectively. In the case of a secondary aromatic amine, however, there must be a molar proportion of amine reactant to tetrakis(halomethyl)methane reactant of about 4:1, respectively. In general, there must be at least enough equivalents of hydrogen supplied by the amine to react with all of the halogen equivalents of the halogen compound reactant.

The temperature of the reaction is a critical factor. In general, satisfactory reaction products are produced at temperatures varying between about 180° C. and about 240° C. It is preferred, however, to operate in a temperature range of from about 215° C. to about 230° C. Reaction products produced at temperatures higher than about 240° C. are ineffective for the purposes of this invention.

The time of the reaction is not a critical factor. It will vary dependent upon the particular reactants involved and upon the reaction temperatures selected. The reaction is carried out until all of the halogen atoms in the tetrakis(halomethyl)methane reactant have combined with hydrogen atoms. In general, the reaction is complete in between about 3 hours and about 15 hours.

In order to ensure complete reaction, the hydrogen halides formed as by-products in the reaction of this invention should be removed by means of a hydrogen halide acceptor. Such an acceptor can be an inorganic base or a tertiary amine. Since the amine reactant used in the present reaction can itself combine with, i. e., "accept," a hydrogen halide, the acceptor must be a stronger base than the amine reactant. As those skilled in the art will recognize, the relative strength of basic materials can be readily determined on the basis of ionization constant data. In any given pair, the base having the higher ionization constant (K) is the more basic. For example, for aniline the value of K is  $3.83 \times 10^{-10}$ , whereas tributylamine has an ionization constant of  $2.1 \times 10^{-4}$ . Since the tributylamine has the higher ionization constant, it follows that it can be used as an acceptor in a reaction involving aniline. This has proven to be the fact, in actual practice. The ionization constants can be readily determined by well known methods. Many values are available in tables, for example in Lange's Handbook of Chemistry and from sources set forth therein. Non-limiting examples of hydrogen halide acceptors utilizable herein are triethylamine, ethyldiisopropylamine, triisopropylamine, amylidopropylamine, triethylamine, triisobutylamine, dimethylbenzylamine, triamylamine, trioctylamine, pyridine, piperidine, caffeine, tetramethylethylenediamine, sodium carbonate, sodium bicarbonate, and sodium acetate. At least sufficient acceptor to react with all of the hydrogen halide produced

70

75

80

in the reaction must be used, i. e., at least 4 moles of hydrogen halide acceptor per mole of tetrakis(halomethyl)-methane. In practice, it is preferable to use a molar excess of hydrogen halide acceptor. Generally, between about 4.1 moles and about 5 moles of acceptor will be used per mole of tetrakis(halomethyl)methane. As will be readily understood by those skilled in the art, in some instances an excess of the amine reactant can be used as a hydrogen halide acceptor. When four moles of a primary or secondary amine are reacted per mole of tetrakis(halomethyl)methane reactant, the reactant amine can be used as an acceptor. Thus, a molar proportion of 8:1 or higher can be employed; four moles of amine for the reaction product production, and the other four moles as the hydrogen halide acceptor.

The reaction of this invention can be carried out either in an open reactor or in a closed reactor. It is preferred, however, to conduct the reaction in a sealed reactor, in order to exclude atmospheric moisture. It has been found that the presence of small amounts of water in the reaction system makes it difficult to attain the temperatures required for the reaction.

The constitution of the reaction products of this invention is not known. It could be postulated, in view of the usual mechanisms of condensation reactions between amines and alkyl halides, that the amine reactant simply replaces the halogen atoms of the tetrakis(halomethyl)methane reactant. This does not appear to be the case, however. The reaction products of the present invention have molecular weights which are higher than the theoretical molecular weights for such a reaction. On the other hand, the molecular weights are lower than those of dimers or other polymerized products. Apparently, the reaction or series of simultaneous reactions involved affords reaction products of a relatively complex nature. Accordingly, it will be appreciated that any definition of the reaction products of this invention, other than a definition comprising the method for making them, is highly inaccurate and non-descriptive.

The following combinations will serve as non-limiting examples of the pairs of reactants which will form the reaction products contemplated herein. In the interests of brevity, molar proportions are indicated by inserting the number of moles of a reactant used in parentheses following its name. Thus, aniline(2)+tetrakis(bromomethyl)methane(1) indicates the reaction product between aniline and tetrakis(bromomethyl)methane in a molar proportion of 2:1, respectively. Non-limiting examples of pairs of reactants are: aniline(3)+tetrakis(chloromethyl)methane(1); 1-naphthylamine(4)+tetrakis(bromomethyl)methane(1); p-toluidine(2)+tetrakis(chloromethyl)methane(1); 4-butyl-1-phenanthrylamine(3)+tetrakis(iodomethyl)methane(1); 9-phenanthrylamine(4)+tetrakis(bromomethyl)methane(1); N-methyl-4-anthrylamine(4)+tetrakis(bromomethyl)methane(1); o-toluidine(3)+tetrakis(chloromethyl)methane(1); 1-anthrylamine(2)+tetrakis(iodomethyl)methane(1); p-ethylaniline(4)+tetrakis(chloromethyl)methane(1); N-isopropyl-3-sec-butyl-1-anthrylamine(4)+tetrakis(bromomethyl)methane(1); 4-propyl-1-anthrylamine(2)+tetrakis(chloromethyl)methane(1); 5-methyl-2-anthrylamine(3)+tetrakis(iodomethyl)methane(1); o-isopropylaniline(4)+tetrakis(iodomethyl)methane(1); p-sec-butylaniline(2)+tetrakis(bromomethyl)methane(1); o-amyylaniline(3)+tetrakis(chloromethyl)methane(1); 4-butyl-1-naphthylamine(4)+tetrakis(iodomethyl)methane(1); N-ethylaniline(4)+tetrakis(chloromethyl)methane(1); N-t-butylaniline(4)+tetrakis(iodomethyl)methane(1); N-isoamyylaniline(4)+tetrakis(bromomethyl)methane(1); N-propyl-4-methyl-1-naphthylamine(4)+tetrakis(bromomethyl)methane(1); N-methyl-o-butylaniline(4)+tetrakis(chloromethyl)methane(1); N-ethyl-2-naphthylamine(4)+tetrakis(iodomethyl)methane(1); N-t-ethyl-2-naphthylamine(4)+tetrakis(iodomethyl)methane(1); N-t-amyl-p-isopropylaniline(4)+tetrakis(bromomethyl)methane(1); N-ethyl-p-toluidine(4)+tetrakis(chloromethyl)methane(1); and N-propyl-m-toluidine(4)+tetrakis(iodomethyl)methane(1).

Separation of the reaction products of this invention is readily effected by methods well known to those skilled

in the art. It is, of course, necessary to remove the hydrogen halide acceptor and the hydrogen halide. Suitably, the hydrogen halide can be removed by extracting the reaction mixture with a strong solution of caustic, such as sodium or potassium hydroxide. In some instances, the amine hydrohalide formed from the addition of an amine acceptor with hydrogen halide can be removed by filtration. The reaction products of the present invention are relatively high-boiling. Accordingly, organic hydrogen halide acceptors can be removed by distillation methods. Steam distillation and distillation under reduced pressure are suitable methods. After removal of the acceptor, hydrogen halide, and the like, it is desirable, though not essential, to extract the residual reaction product with a water-insoluble solvent, in order to isolate the reaction product from inorganic salts and the like. Suitable solvents are diethyl ether, benzene, chloroform, toluene, xylene, etc. The extracts can be combined and evaporated or distilled to remove the solvent, thus leaving the desired reaction product. As indicated hereinbefore, however, this step is not necessary. The residual reaction product remaining in the distillation vessel is utilizable as such, provided the caustic material, inorganic salts, etc., are removed by other methods, such as by a washing operation.

The following specific examples are for the purpose of exemplifying and illustrating the present invention. It is to be strictly understood, however, that the invention is not to be limited to the specific reactants set forth in these examples, or to the operations and manipulations described therein. As will be apparent to those skilled in the art, a wide variety of other reactants, as set forth hereinbefore, can be used to prepare the products contemplated herein.

#### EXAMPLE 1

##### Reaction of aniline (2) with tetrakis(bromomethyl)-methane(1) in an open vessel

A mixture of 19.4 grams (0.05 mole) of tetrakis(bromomethyl)methane, 9.3 grams (0.1 mole) of aniline, and 46 grams (0.25) mole of tri-n-butylamine were placed in a reaction flask equipped with a thermometer and a reflux condenser. The mixture was heated at refluxing temperatures for 9 hours. During the reaction period, the temperature of the reaction mixture rose from 180° C. to 226° C. The reaction mixture was cooled and then made strongly alkaline by the addition of 400 milliliters of a 5 per cent (weight) aqueous solution of sodium hydroxide. This mixture was then subjected to steam distillation until 7.5 liters of steam distillate had been collected. At this point, there was substantially no organic material coming over with the steam distillate. The residue remaining in the flask was cooled and extracted with about 200 milliliters of diethyl ether. The ether solution was washed with water to remove water-soluble material, and dried over solid potassium hydroxide. The ether solution of the product was filtered. Then the solvent (ether) was removed by evaporation on the steam bath. The product (10.5 grams) was a dark-colored, oil-soluble oily material. It contained 7.48 percent nitrogen and had a molecular weight of 406. The product gave a negative test for halogen.

#### EXAMPLE 2

##### Reaction of aniline (2) with tetrakis(bromomethyl)-methane(1) in a closed reactor

A mixture of 97 grams (0.25 mole) of tetrakis(bromomethyl)methane, 46.5 grams (0.5 mole) of aniline, and 213 grams (1.15 moles) of tri-n-butylamine was placed in a closed bomb and heated at 230±5° C. for 12 hours. After cooling, the semi-solid reaction product was transferred to a distillation vessel and made alkaline with a solution of 52 grams of 97 per cent sodium hydroxide in 300 milliliters of water. As described in Example 1, the mixture was subjected to steam distillation until no appreciable amount of organic matter distilled over. A total of 8.5 liters of steam distillate were collected. The residue was cooled and taken up in about 300 milliliters of diethyl ether. The ether solution was washed with water and then dried over solid potassium hydroxide. The dried solution was filtered. Then, the ether was removed by evaporation on the steam bath, leaving 55 grams of a dark-colored oil as the reaction product. This

product contained 7.21 per cent nitrogen, had a molecular weight of 406, and contained no halogen.

### EXAMPLES 3 THROUGH 7

Five reaction products were prepared, using the procedure described in Example 2, by reacting tetrakis(bromomethyl)methane with different aromatic amine reactants, in several molar proportions and at various temperatures. Pertinent data for these runs and for the reaction products obtained are set forth in Table I.

TABLE I

| Exam-<br>ple | Moles of Amine per Mole<br>of Tetrakis(bromomethyl)<br>methane | Reac-<br>tion<br>Time,<br>Hours | Reac-<br>tion<br>Tem-<br>pera-<br>ture,<br>° C. | Product Anal-<br>ysis |                          |
|--------------|----------------------------------------------------------------|---------------------------------|-------------------------------------------------|-----------------------|--------------------------|
|              |                                                                |                                 |                                                 | Per-<br>cent<br>N     | Mole-<br>cular<br>Weight |
| 3            | Aniline, 4 moles                                               | 12                              | 230±5                                           | 8.81                  | 414                      |
| 4            | p-Toluidine, 2 moles                                           | 12                              | 260±5                                           | 6.01                  | 325                      |
| 5            | p-Toluidine, 2 moles                                           | 12                              | 230±5                                           | 7.07                  | 570                      |
| 6            | p-t-Amyl aniline, 2 moles                                      | 12                              | 230±5                                           | 5.74                  | 360                      |
| 7            | N-Ethylaniline, 4 moles                                        | 12                              | 230±5                                           | 8.30                  | 458                      |

Two base oils were used in evaluating the reaction products aforescribed. Base oil A is a solvent refined Mid-Continent (Rodessa) distillate stock having a specific gravity of 0.860, a flash point of 405° F., and a viscosity of 155 S. U. S. at 100° F. Base oil B is an acid-refined Mid-Continent distillate stock having a specific gravity of 0.879, a flash point of 385° F., and a viscosity of 152 S. U. S. at 100° F. Both of these oils are suited for use in steam turbines.

### EXAMPLE 8

The reaction products prepared as described in Examples 1 through 7 were subjected to the Brown-Boveri Turbine Oil Test. This test is described in the Brown-Boveri Rev., 16 (2), 92-7 (1929). In brief, a 200-milliliter sample of oil under test is placed in a 400-milliliter covered beaker containing a V-shaped piece of polished copper. Air is passed over the surface of the oil at a rate of two liters per hour. The test is carried out for 72 hours at 230° C. and then for 24 hours at room temperature. The results, in terms of condition of the copper, neutralization number (N. N.), and Lovibond color, indicate the oxidation stability of the oil tested. These results are compared with similar results for the uninhibited base oil. Pertinent test results for the reaction products of Examples 1 through 7 are set forth in Table II.

TABLE II  
[Brown-Boveri Turbine Oil Test.]

| Additive  | Wt. Per-<br>cent<br>Conc. | Results in Base Oil A  |                    |        | Results in Base Oil B  |                    |        |
|-----------|---------------------------|------------------------|--------------------|--------|------------------------|--------------------|--------|
|           |                           | Lovi-<br>bond<br>Color | N. N. <sup>1</sup> | Copper | Lovi-<br>bond<br>Color | N. N. <sup>1</sup> | Copper |
| None      |                           | 58                     | 0.19               | O. K.  | 8                      | 0.07               | O. K.  |
| Example 1 | 0.2                       | 2.5                    | 0.02               | O. K.  | 2.5                    | 0.03               | O. K.  |
| Example 2 | 0.2                       | 9.0                    | 0.01               | O. K.  | 12                     | 0.07               | O. K.  |
| Example 3 | 0.2                       | 5.0                    | 0.02               | O. K.  | 9                      | 0.02               | O. K.  |
| Example 4 | 0.2                       | 16.0                   | 0.01               | O. K.  | 40                     | 0.47               | O. K.  |
| Example 5 | 0.2                       | 7.0                    | 0.05               | O. K.  | 12                     | 0.05               | O. K.  |
| Example 6 | 0.2                       | 90.0                   | 0.78               | Bright | 46                     | 0.60               | O. K.  |
| Example 7 | 0.2                       | 1.3                    | 0.03               | O. K.  | 4                      | 0.05               | O. K.  |

<sup>1</sup> Neutralization number.

### EXAMPLE 9

Some of the reaction products described in the preceding examples were subjected to the ASTM Turbine Oil Oxidation Test. This test is fully described in the ASTM Manual as Test D-943-47T. In general, the test involves placing a 300-milliliter sample of test oil in a tube provided with a gas inlet having a fritted glass outlet, and a catalyst coil consisting of interwound iron and copper wire. The test is conducted at a temperature of 203±0.9° F. Sixty milliliters of water are maintained in the tube, and oxygen is passed through the oil at the rate of three liters per hour. The test is continued until period testing shows that the oil has greatly increased

in acidity, a sign of the formation of acidic oxidation products. These data are usually plotted graphically. Color can also be noted, although acidity is the primary criterion in this test.

- 5 In addition to the uninhibited base oils A and B, four other blends were tested in this test. Blend R was a blend of 0.2 weight per cent of the reaction product of Example 1 in base oil A. Blend S was a blend of 0.2 per cent of the same reaction product in base oil B. 10 Blend T was a blend of 0.2 weight per cent of the reaction product of Example 3 in base oil A. Blend U consisted of 0.2 per cent, by weight, of the reaction product of Example 7 in base oil A. Pertinent data for these runs are set forth in Table III.

TABLE III  
[ASTM Turbine Oil Oxidation Test Results.]

| Blend | Blend Data | Hours | Days | Lovi-<br>bond<br>Color | N. N. <sup>1</sup> |
|-------|------------|-------|------|------------------------|--------------------|
|       |            |       |      |                        |                    |
| 20    | Base Oil A | 24    | 1    | 3                      | 0.05               |
|       |            | 48    | 2    | 14                     | 0.92               |
|       |            | 72    | 3    | 172                    | 5.1                |
| 25    | Base Oil B | 120   | 5    | 7                      | 0.02               |
|       |            | 144   | 6    | 1.8                    | 0.08               |
|       |            | 168   | 7    | 5                      | 0.55               |
|       |            | 194   | 8    | 16                     | 1.9                |
|       |            | 219   | 9    | 32                     | 3.2                |
|       |            | 1,920 | 80   | 2                      | 0.04               |
|       |            | 2,952 | 123  | 2.5                    | 0.02               |
| 30    | Blend R    | 4,176 | 174  | 4                      | 0.06               |
|       |            | 4,848 | 202  | 8.7                    | 0.70               |
|       |            | 4,944 | 206  | 78                     | 5.7                |
|       |            | 1,584 | 66   | 13                     | 0.24               |
|       |            | 1,776 | 74   | 19                     | 0.42               |
|       | Blend S    | 1,920 | 80   | 22                     | 0.65               |
|       |            | 2,016 | 84   | 25                     | 0.88               |
|       |            | 2,112 | 88   | 52                     | 1.4                |
| 35    |            | 2,256 | 94   | 285                    | 14.1               |
|       |            | 1,848 | 77   | 8                      | 0.04               |
|       | Blend T    | 2,352 | 98   | 8                      | 0.04               |
|       |            | 3,552 | 148  | 9                      | 0.08               |
|       |            | 4,512 | 188  | 12                     | 0.06               |
| 40    |            | 1,848 | 77   | 6                      | 0.06               |
|       | Blend U    | 2,352 | 98   | 6                      | 0.04               |
|       |            | 3,552 | 148  | 6                      | 0.06               |
|       |            | 4,272 | 178  | 9                      | 0.4                |
|       |            | 4,368 | 182  | 16                     | 2.8                |

45 <sup>1</sup> Neutralization number.

In the figure, the acidity (N. N.) data for the runs reported in Table III are plotted graphically. As will be apparent from the curves for oils A and B, the uninhibited oils rapidly undergo oxidation. The curves therefore are typical; in that the acidity of the oil remains low until oxidation commences. At that point, acidity in-

creases rapidly, often within a matter of a few hours. It will be noted that test blend R (0.2 per cent Example 1 in oil A) maintained a low acidity for 200 days. It was not until over 200 days (not shown) that the rate of oxidation had increased to the point that acidic bodies had been formed to an appreciable extent. The blend of acid refined base oil B containing 0.2 per cent of the product of Example 1 lasted for almost 90 days, before its acidity increased tremendously. As is well known to those familiar with the art, acid refined oils are much more difficult to inhibit than are solvent refined oils. Accordingly, the difference in response of oils A and B to the same additive is to be expected. Test blend T

(0.2 per cent of product of Example 3 in base oil A) had an extremely low N. N. even at 188 days and showed no signs of becoming oxidized. The blend of 0.2 per cent of the product of Example 7 in base oil B (Curve U) lasted for about 180 days before it showed appreciable acidity.

In the foregoing examples, the preparation and the effectiveness of the reaction products of this invention have been demonstrated. It will be appreciated that these products are excellent stabilizers for lubricating oils. Also, it will be noted that they are effective in stabilizing both solvent refined oils and acid refined oils against oxidation.

The amount of the reaction products of this invention which is blended with a mineral lubricating oil varies between about 0.05 per cent and about 5 per cent, by weight. It is ordinarily preferred to use between about 0.1 per cent and about 2 per cent, by weight. Concentrates of these reaction products in mineral oils are contemplated. Accordingly, more than 5 per cent, and up to 49 per cent of the reaction products (limited by the dispersibility thereof in mineral oil) might be blended in a mineral oil, which oil need not be the same type of oil that is ultimately used. Thus, a concentrate can be prepared in a light oil, such as a kerosene or light household oil. The concentrate can then be dissolved, in the requisite amount, in the oil to be inhibited, in order to achieve a blend containing the desired amount of additive.

Other oil addition agents can be used in conjunction with the additives of this invention, to improve other properties of the oil. For example, antirust agents, oiliness agents, V. I. improvers, pour point depressants, detergents, antifoamants, E. P. agents and the like can be added to the lubricating oil along with the additives of this invention. Such other additives are well known to those familiar with the art. Accordingly, it is believed unnecessary to list them here.

Although the present invention has been described with preferred embodiments, it is to be understood that modifications and variations may be resorted to without departing from the spirit and scope thereof, as those skilled in the art will readily understand. Such variations and modifications are considered to be within the purview and scope of the appended claims.

What is claimed is:

1. A mineral lubricating oil containing a small amount, sufficient to inhibit the oxidation tendencies thereof, of the reaction product obtained by reacting (1) a tetrakis(halomethyl)methane of the general formula:



55

wherein X is selected from the group consisting of bromine, chlorine and iodine, with (2) an amine having the general formula  $\text{HRNYR}'$  wherein Y is a benzene nucleus, R is a radical selected from the group consisting of hydrogen and an alkyl radical having from one to 5 carbon atoms, and R' is a radical selected from the group consisting of hydrogen and an alkyl radical having from one to 5 carbon atoms and having at least one hydrogen atom attached to the carbon atom thereof which is attached to the aromatic nucleus, at a temperature of from about 180° C. to about 240° C.; the proportion of said amine to said tetrakis(halomethyl)methane utilized in the reaction being from about 2 to about 4 mols of said amine per mol of said tetrakis(halomethyl)methane when the radical R in said amine is hydrogen and about 4 mols of said amine per mol of said tetrakis(halomethyl)methane when the radical R in said amine is alkyl.

2. A mineral lubricating oil containing between about 0.05 per cent and about 5 per cent, by weight, of the reaction product obtained by reacting (1) a tetrakis(halomethyl)methane of the general formula:



80

wherein X is selected from the group consisting of bromine, chlorine and iodine, with (2) an amine having the general formula  $\text{HRNYR}'$  wherein Y is a benzene nucleus, R is a radical selected from the group consisting of hydrogen and an alkyl radical having from one to 5 carbon atoms and having at least one hydrogen atom attached to the carbon atom thereof which is attached to the aromatic nucleus, at a temperature of from about 180° C. to about 240° C.; the proportion of said amine to said tetrakis(halomethyl)methane utilized in the reaction being from about 2 to about 4 mols of said amine per mol of said tetrakis(halomethyl)methane when the radical R in said amine is hydrogen and about 4 mols of said amine per mol of said tetrakis(halomethyl)methane when the radical R in said amine is alkyl.

5 10 15 20 25 30 35 40 45 50 55 60 65 70 75 80 85

8 The reaction product obtained by reacting a tetrakis(bromomethyl)methane with aniline, in a molar proportion of said aniline to said tetrakis(bromomethyl)methane of about 2:1, respectively; and at a temperature of between about 180° C. and about 240° C.

9. A mineral lubricating oil containing a small amount, sufficient to inhibit the oxidation tendencies thereof, of the reaction product obtained by reacting tetrakis(bromomethyl)methane with aniline, in a molar proportion of said aniline to said tetrakis(bromomethyl)methane of about 2:1, respectively; and at a temperature of between about 180° C. and about 240° C.

10 15 20 25 30 35 40 45 50 55 60 65 70 75 80 85

10. A mineral lubricating oil containing a small amount, sufficient to inhibit the oxidation tendencies thereof, of the reaction product obtained by reacting a tetrakis(bromomethyl)methane with aniline, in a molar proportion of said aniline to said tetrakis(bromomethyl)methane of about 2:1, respectively; and at a temperature of between about 180° C. and about 240° C.

11 16 21 26 31 36 41 46 51 56 61 66 71 76 81 86

11. A mineral lubricating oil containing a small amount, sufficient to inhibit the oxidation tendencies thereof, of the reaction product obtained by reacting tetrakis(bromomethyl)methane with p-toluidine, in a molar proportion of said p-toluidine to said tetrakis(bromomethyl)methane of about 2:1, respectively; and at a temperature of between about 180° C. and about 240° C.

12 17 22 27 32 37 42 47 52 57 62 67 72 77 82 87

12. A mineral lubricating oil containing a small amount, sufficient to inhibit the oxidation tendencies thereof, of the reaction product obtained by reacting a tetrakis(bromomethyl)methane with N-ethylaniline, in a molar proportion of said N-ethylaniline to said tetrakis(bromomethyl)methane of about 4:1, respectively; and at a temperature of between about 180° C. and about 240° C.

13 18 23 28 33 38 43 48 53 58 63 68 73 78 83 88

13. The reaction product obtained by reacting (1) a tetrakis(halomethyl)methane of the general formula:



55

wherein X is selected from the group consisting of bromine, chlorine and iodine, with (2) an amine having the general formula  $\text{HRNYR}'$  wherein Y is a benzene nucleus, R is a radical selected from the group consisting of hydrogen and an alkyl radical having from one to 5 carbon atoms and having at least one hydrogen atom attached to the carbon atom thereof which is attached to the aromatic nucleus, at a temperature of from about 180° C. to about 240° C.; the proportion of said amine to said tetrakis(halomethyl)methane utilized in the reaction being from about 2 to about 4 mols of said amine per mol of said tetrakis(halomethyl)methane when the radical R in said amine is hydrogen and about 4 mols of said amine per mol of said tetrakis(halomethyl)methane when the radical R in said amine is alkyl.

14 19 24 29 34 39 44 49 54 59 64 69 74 79 84 89

14. The reaction product obtained by reacting a tetrakis(bromomethyl)methane with aniline, in a molar proportion of said aniline to said tetrakis(bromomethyl)methane of about 4:1, respectively; and at a temperature of between about 180° C. and about 240° C.

15 20 25 30 35 40 45 50 55 60 65 70 75 80 85

15. The reaction product obtained by reacting a tetrakis(bromomethyl)methane with p-toluidine, in a molar proportion of said p-toluidine to said tetrakis(bromomethyl)methane of about 4:1, respectively; and at a temperature of between about 180° C. and about 240° C.

methane of about 2:1, respectively; and at a temperature of between about 180° C. and about 240° C.

11. The reaction product obtained by reacting a tetrakis(bromomethyl)methane with N-ethylaniline, in a molar proportion of said N-ethylaniline to said tetrakis(bromomethyl)methane of about 4:1, respectively; and at a temperature of between about 180° C. and about 240° C.

## References Cited in the file of this patent

## UNITED STATES PATENTS

|   | Number    | Name         | Date          |
|---|-----------|--------------|---------------|
| 5 | 2,451,642 | Watson ----- | Oct. 19, 1948 |
|   | 2,530,769 | Hollis ----- | Nov. 21, 1950 |